

G. A. HENDERSON,  
PAVEMENT AND PROCESS OF MAKING THE SAME,  
APPLICATION FILED JAN. 15, 1918.

1,370,815.

Patented Mar. 8, 1921.

4 SHEETS—SHEET 1.



Witnesses:

W. H. H. *W. H. H.*  
H. H. H. *H. H. H.*  
H. H. H. *H. H. H.*

## *Inventor:*

George A. Hinckley

G. A. HENDERSON.

PAVEMENT AND PROCESS OF MAKING THE SAME.  
APPLICATION FILED JAN. 15, 1918.

1,370,815.

Patented Mar. 8, 1921.

4 SHEETS—SHEET 2.



*Inventor:*

George A.  
Henderson

Urgencies:  
Orardian W.W. W.

G. A. HENDERSON,  
PAVEMENT AND PROCESS OF MAKING THE SAME,  
APPLICATION FILED JAN. 15, 1918.

1,370,815.

Patented Mar. 8, 1921.

4 SHEETS—SHEET 3.



G. A. HENDERSON,  
PAVEMENT AND PROCESS OF MAKING THE SAME,  
APPLICATION FILED JAN. 15, 1918.

1,370,815.

Patented Mar. 8, 1921.

4 SHEETS—SHEET 4.



*Fig. 9.*

Witnesses:

O. H. Anderson  
Minneapolis.

Inventor:  
George A. Henderson

# UNITED STATES PATENT OFFICE.

GEORGE A. HENDERSON, OF ST. ALBANS, WEST VIRGINIA, ASSIGNOR TO THE BITUMINOUS CONCRETE COMPANY OF AMERICA, OF CHARLESTON, WEST VIRGINIA, A CORPORATION OF WEST VIRGINIA.

## PAVEMENT AND PROCESS OF MAKING THE SAME.

1,370,815.

Specification of Letters Patent.

Patented Mar. 8, 1921.

Application filed January 15, 1918. Serial No. 212,194.

To all whom it may concern:

Be it known that I, GEORGE A. HENDERSON, a citizen of the United States, residing at Highland Villa, at St. Albans, in the county of Kanawha and State of West Virginia, have invented certain new and useful Improvements in Pavements and Processes of Making the Same, of which the following is a specification.

10 My invention relates to a combination of the two types of pavements characterized and known to the trade as "bituminous macadam", having a wearing course of broken stone with some interstitial spaces filled 15 by penetration methods with a bituminous binder, and as "bituminous concrete", composed of stone, gravel, sand, shell, slag, or other aggregate, or combinations thereof, and bituminous materials, incorporated together by mixing methods; and relates to substantial departure from the ordinary methods and from the apparatus heretofore used in such construction, in various particulars which will be more fully exemplified 20 and set forth in the subjoined detailed specification.

The invention particularly relates to resurfacing macadam roads to a substantial thickness of mixed and bonded material, 30 the major portion of the mineral aggregate in which is composed of the old road, with which a comparatively small quantity of new material is mixed in cases where traffic has left a sufficient quantity of metal over an 35 adequate sub-base for the purpose of increased traffic to be attracted by the improved structure, and the object of my invention is the economical correction of conditions in the prior art relating to paving 40 structures, the sanitary removal of dust from the surface of a highway, as well as from its internal structure, to be reincorporated and retained therein suspended in bitumen.

In carrying out my invention a road's 45 surface is broken, then scarified, and, during heating of the surface to a substantial depth, the surface and internal dust is removed and the remaining aggregate, in its loose, ridged, heated and dustless condition, is 50 coated, during turning, with bitumen uniformly distributed, under pressure, sufficient to also cause penetration of the remaining aggregate on the roadway, to which surface is immediately added new material consist-

ing of a graded aggregate coated with pre-heated bitumen in the absence of dust during 55 drying and heating of such aggregate, which is then mixed with preheated dust coated in hot air suspension under sustained heat with preheated atomized bitumen, then raked and 60 pressed into the interstitial spaces between the larger particles of loose stone on the road, in merely sufficient quantity to fill them.

My invention will be best understood by 65 reference to the accompanying drawings, which will now be described, it being premised however, that various changes may be made in the apparatuses by which the same may be operated and the process carried out, 70 without departing from the spirit and scope of the appended claims.

Figure 1 is a view partly in side elevation and partly in vertical section of apparatus adapted for carrying out the invention; Fig. 75 2 is a cross sectional front end view, and Fig. 3 a cross sectional rear end view thereof. Fig. 4 is a top cross sectional view of the machine and of a roadway under its treatment; Fig. 5 illustrates a pavement 80 in vertical section before reconstruction, in which "a" is dust, "b" is stone and "c" is earth; Fig. 6, a similar section after it is scarified and the interstitial dust removed, in which "a" is dust, "b" stone, and "c" 85 earth; Fig. 7 a similar section after a bituminous compound has been added thereto, in which "a" is dust, "b" stone, "c" earth and "d" bitumen; Fig. 8 a similar section of pavement reconstructed in accord with 90 this invention, in which "a" represents relatively small sizes of stone coated with bitumen and mixed with bituminized dust, "b" is the bitumen coated stone shown in Fig. 7, "c" is earth, and "a" is unremoved 95 dust in the lower section of the pavement penetrated with bitumen. Fig. 9 is a cross sectional view, representing the entire width of a highway reconstructed in accord with this invention, in which "F" is the material 100 shown in Fig. 8, "G" "G" shoulders thereto constructed by the ordinary penetration method, or added stone aggregate, and "C", "C" earth.

In instances where the highway is completely reconstructed fourteen feet or more in width, temporary steel curbing "f" shown in Figs. 1 and 3 constitute two sides

of the "furnace" hereinafter described, the surface to be treated in one operation being seven feet wide, the remaining width being opened to traffic meanwhile. In such instance rear side wheels "S" "S" in Fig. 3 travel outside of the area inclosed by the curbing "f<sup>5</sup>". In instances where the center of a country road is to be so completely reconstructed seven feet in width (to which width from one and a half to three and a half feet of metal shoulders shall be added to each side) multipedal or caterpillar traction units are designed to constitute such furnace sides and support the rear of the machine in lieu of its side wheels "S", "S" in Fig. 3.

The entire machine is designed to travel over the surface under reconstruction at a speed predetermined and automatically fixed by moving members operating the machine's internal mechanism consistent with its capacity and the area of the pavement under construction. To illustrate, on the basis of a machine whose capacity is 1000 sq. yds. of 2" compressed new material per eight-hour day, (passing out of the drum hereinafter described), which material, representing substantially one-third of the "bituminous-concrete" surface constructed in the operation, is pressed into said interstices of the remaining two-thirds of material left on the road on the basis of approximately  $\frac{3}{4}$ " of thickness of such added material, the machine, in constructing a strip of highway seven feet wide by 3428 feet long in eight hours shall travel at the rate of approximately 428 feet per hour, and subject all parts of such surface to the hot blasts hereinafter described for the period of approximately two minutes, the length of the furnace and drum being approximately fifteen feet.

In reconstructing a country road, with main traffic center seven feet in width, widened to from ten to fourteen feet in wearing surface, width, in the manner hereinafter described; the old surface is not necessarily "brought to crown" or otherwise treated except to provide adequate side drainage; the added center material, shaped off by penetration method shoulders has been found to be adequate in this regard. Substantial depressions are completely filled with untamped, cold stone preferably of the character of which the old road was constructed; the roadway is not swept, the dust being handled by the machine which simultaneously burns the combustible material therein as well as that leached to the interstices. Freshly deposited manure and the larger particles of foreign matter that may be present on the road shall be removed, ahead of the machine, manually.

Referring, now, to Figs. 1 and 2, I-beam 65 "J" and front pivot and rear axle supports

"j" "j" constitute the frame work of the machine, properly braced, front supporting roller "j" having a spiked tread the width of which is that of the machine and designed to partially break the old surface of the highway. The sufficient weight of the entire machine, in its powerful course forward, causes tines "b" "b" under control of the operator, in the use of lever "t", to scarify in the first instance, and to turn, the stone in the road during treatment thereof as hereinafter described. Immediately following the forward of the three sets of tines "b" "b" "b", the forward set of fuel burners d' d' supplied under sufficient air pressure with oil from forward auxiliary equipment, through supply pipe "d", are designed to throw downwardly and backwardly a blast of flame (x x) equivalent to approximately 1500 cu. ft. per minute capacity, later augmented by (a) like burners of approximately 1000 cu. ft. capacity per minute, which may be faced downwardly and forward, and connected with the supply pipe "d" extending through the longitudinal center of the furnace, and (b) the sheet blast of hot air from drum "7" hereinafter referred to.

The furnace consists of a bottom, to-wit: the road's surface; the furnace top consists of the bottom of the bitumen tank "k"; its sides consists of said multipedal units or temporary curbing f<sup>5</sup> anchored to the pavement by spikes f<sup>6</sup> designed to be removed after compression of the completed pavement, and relaid ahead of the machine, such sides having overlapping members "e" "e" with lateral springs e', which overlapping members "e" "e" and curb f<sup>5</sup> are designed to carry no part of the weight of the machine, or to guide it, but are designed to eliminate lateral suction of cold air to the furnace, and to retain the elevated surface caused by scarifying.

The dust and fine particles, in quantity exceeding fifteen per cent. of the aggregate, 110 ranging from those that will pass a 80-holes to the linear inch screen to those substantially smaller than those that pass a screen of 200 mesh to the linear inch, are loosened by (a) the forward roller spikes, (b) the scarifiers and (c) the aforesaid hot blasts, as well as by suction through fans C' C' C' and C' (Fig. 2) revolved by belt and pulley connections C<sup>1</sup> C<sup>2</sup> shown in detail in Fig. 3. Such dust and fines are thereby 115 lifted from the surface of the highway, through screens (shown in Fig. 4) at the mouth of flues f<sup>2</sup> f<sup>2</sup> (shown in Fig. 1) penetrating bitumen tank "k" and passed through continuation of flues f<sup>2</sup>, to-wit: 120 flues f<sup>3</sup> and f<sup>4</sup>, then through fan C', in a cloud to and within mixing drum "7" anchored within the lines of tank "k," and therein surrounded, (with the exception of its ends) with hot bitumen, which from an 125

auxiliary supply tank, is, in said tank "k" further heated after reaching it, through intake "p" (preferably asbestos covered) under pressure, which heat in tank "k" is supplied by the furnace at its bottom and through flues  $f^2$  aforesaid. An approved thermometer, anchored in sight of the operator, is set within the metal of tank "k" and the temperature of the bitumen therein is regulated by adjusting the supply to fuel oil burners  $d$  aforesaid. The bitumen in tank "k" is designed to be constantly agitated by suction through pump "o" with indicator  $o'$  through intake pipe "n" and outlet pipe  $n^2$ , which is designed to supply the flow of bitumen to and within the forward end of drum  $l$ , through cock  $n^4$  and indicator  $n^5$  in predetermined quantity under control of an operator there seated, which quantity is fixed consistent with the quantity of clean, cold stone which passes from hopper Q through gate Q' (Fig. 1), which gate is automatically revolved by cogged wheels M' (Fig. 1) anchored to main motor-driven shaft  $m$ , at a speed fixed consistent with the capacity of drum  $l$ , as determined by its size and the speed at which material therein may be manipulated by agitators  $l'$  set at angles to form a perfect screw therein, to agitate and push the material from the forward to its rear end, while mixing, and out at gate  $l^4$ , automatically revolved by connection at the rear end of main shaft  $m$  with cogs  $m^3$ . Bitumen agitating pipe  $n^2$  extends to and within the bitumen tank  $k$  near its forward end and on the reverse side of drum  $l$  from its intake  $n$ , and interposed between the pump  $o$  and mouth is hand operated cock N $^4$  and connections for withdrawing bitumen for said prescribed purposes.

The hot bitumen surrounding drum  $l$  is designed to heat drum  $l$  externally, and to thereby heat its contents in addition to the heat thereto applied directly internally through flues  $f^2$  and  $f^3$  aforesaid, for the purpose of subjecting the mixture therein to sustained heat sufficient in duration and temperature, consistent with the capacity of the machine to not only, during agitation and mixing, coat the clean stone screenings with hot bitumen, but to evaporate in the form of steam, any moisture contained in such stone, to be removed from drum  $l$  as hereinafter described.

In this connection be it remembered that moisture becomes steam at a temperature of 212 degrees Fahr., and at that temperature is exceeding 1000 times its volume as water; that in ordinary paving mixtures bitumen is deposited on preheated stone at a temperature of from 300 to 350 degrees Fahr. and that in this process, as in the prior art, it is designed that the mixture shall be deposited on to the road at an average

temperature of 250 degrees Fahr. I, accordingly, have discovered that by entrapping a limited moisture content in cold stone surrounded by hot bitumen such moisture may be more advantageously, than otherwise, eliminated through the bitumen under heat sustained sufficient for the purpose after such damp, cold stone has come in contact with the molten bitumen, provided that this is done under suction in an otherwise inclosed drum, wherein the ingredients are deposited to substantially one-third of the drum's capacity, (if figured cold) and continuing the mixing operation therein under sustained heat sufficiently applied to develop and to exhaust the absorbing capacity of the aggregate during elimination of the moisture content. I have discovered that the moisture, acting as a carrying agent of the bitumen, during ebullition thereof, not only coats the particles with the carried bitumen, during evolution of the moisture into steam, but that the aggregate is thoroughly dried and uniformly coated without danger of burning it or the bitumen, especially when this is done in a drum, the heat surrounding and within which is so perfectly regulatable as by the means herein disclosed.

Before the mass has been agitated by the forwarding blades or agitators  $l'$ , anchored to driven shaft  $M$  revolved by motor connection at the bearing  $M'$  at front of the machine, to the extent that such mass has gone midway between the front and rear of drum  $l$ , each particle of such dustless aggregate is thoroughly dried and uniformly coated with bitumen in the absence of dust. Without the circumferential area of the revolving agitators, and alternating dodge fashion about the top of the rear half of drum  $l$ , bitumen atomizing nozzles  $n^3$  spray in the drum a predetermined quantity of bitumen from supply pipe  $n^2$  passing through the hot bitumen in tank  $k$  from the auxiliary supply pumped thereto through cock  $d^4$  and indicator  $d^5$  under control of the operator.

Detritus and extraneous matter being removed by destructive distillation in the manner described, the remaining dust from the interstitial spaces and surface of the loosened stone on the road is hot before it reaches the inside of drum  $l$  at its rear end in hot air suspension, and in such suspension baffled in said drum by plates practically anchored therein for the purpose; such impalpable dust and small particles passing the 80-mesh to the linear inch screen at the mouths to flues  $f^2$  shown in Fig. 4, is, in said drum entrapped by the atomized bitumen sprayed thereon in such hot air suspension, the air thereby freed from the dust, being then sucked, with steam and fumes from the heating mixture in said drum, through the front end thereof by two powerful suction

fans C' C', shown in Fig. 2, operated by belt and pulley connections operating rear suction fans shown in Figs. 2 and 3.

- The steam laden hot air may then be exhausted into the free air and discarded, or, at the front of the machine as shown in the drawings, this hot air may converge into a sheet blower C C C C, faced downwardly and backwardly, thereby creating a circular current of air in sheet form mixed with the flame blasts, hereinabove described, on to the surface of the highway, back, up and then forward and down again during the machine's forward movement.
- 15 In instances where one strip is designed to be laid in the center of the highway, this sheet blower may have attached to its either side, laterally, an off-set blower, designed to be extended adjustably forward of the machine, for the purpose of blowing from the surface to the sides, of the reconstructed pavement, all dust to and within the vacuum influence of the furnace, in order that such sides surface may be dustless for the purpose of receiving bitumen designed to penetrate it at the rear and to the sides of the machine, and of the reconstructed pavement, through laterally adjustable nozzles, connected with the pressure distributor of hot bitumen, which will now be described.
- On to the loosened, scarified, dustless and heated stone aggregate of sizes larger than 80 to the inch mesh, remaining on the road's surface, illustrated in Fig. 6 hot bitumen 35 from forward auxiliary bitumen heater, passes through cock g<sup>2</sup> and indicator g<sup>3</sup>, in predetermined quantity under control of the operator, and through supply pipe g extending within and backwardly through the fire 40 box or furnace to penetration and spraying nozzles g' at the rear of the machine, where, under pressure from the supply tank forward, this bitumen penetrates the surface of such road material in its heated, dust cleared 45 loose condition, to an extent substantially greater than is possible by methods known to the prior art. The nozzles g' are preferably set dodge fashion on cross pipe g (Figs. 2-3) extending the width of the surface 50 under treatment; and, between such nozzles turning tines b shown in Fig. 1, harrow and again turn the stone during the bitumen's contact therewith, to further facilitate coating of all sizes uniformly.
- 55 At this point it is notable that the new clean stone screenings that go into the drum l through hopper Q, are coated with bitumen without interference of any dust mixed with them and that the interstices are filled with 60 particles ranging from 80 mesh size to those substantially finer than 200 mesh size, (ground to such impalpability by previous traffic on the road and from time to time leached therein) which dust is before reaching 65 the drum preheated in the flame and

hot air suspension under suction, and is then coated with the atomized hot bitumen, in the rear of the drum before admixture with the pre-coated stone screenings, with which they then come into contact and are further 70 mixed and agitated in the drum; likewise the stone on the road is coated with bitumen in the absence of dust or any other interfering agency, (such as dust in its interstices, and the chilling influence of cold stone) it 75 being designed that the interstitial spaces between such road stone shall be filled by compression of the mixture from the drum, added thereto while such road stone is in an uncompressed condition, and the mass then 80 pressed into shape.

It is notable at this point that three different kinds of bitumen may be used in the process, although I do not limit myself to the following advantages of this practice, 85 to-wit: (a) the filler stone screenings may be coated with a hard bituminous cement mixed with a softer ingredient colloidally interposed through stiffening dust to act as a filler between such filler-stone screenings 90 in the interstitial spaces of the larger stone precoated with a different bituminous compound, such operation being economically advantageous in reducing costs of various bitumens, more practically and efficiently 95 usable for the designed purposes than the use of a single ingredient for different purposes.

As the material from drum l emerges in a continuous flow onto the heated and 100 bituminized road surface in its loose, ridged, condition, it is immediately raked by hand to a depth not exceeding one inch in thickness over the bituminized stone on the road, steam roller compression being 105 relied upon to (a) compress and incorporate the smaller aggregate mixture within the interstices of the larger stone on the surface, and (b) to compact such scarified stone into a mass superior in density to any 110 structure of which I have knowledge.

Upon removal of the temporary curbs the completed strip may be painted at its proper edges, with bitumen, and other strips added, or shoulders constructed, as shown 115 in Fig. 9 of the drawings.

I claim:

1. The process of treating a worn highway, in a continuous operation, consisting in breaking, then scarifying its structure and loosening the bond between the aggregate; then applying thereto hot air and flame blasts under pressure to remove the relatively small particles and dust from the interstitial spaces of the scarified material, simultaneously heating, while turning, the same, and sucking, in air suspension, the smaller particles and dust into a preheated drum, simultaneously by destructive distillation removing extraneous matter from 120
- 125
- 130

- the old structure; then by pressure distributors causing a bituminous compound to penetrate the scarified dustless heated stone remaining in the structure to a substantial 5 depth thereof during turning of said stone, at the same time preparing additional material consisting in clean stone screenings containing atmospherically absorbed moisture, which screenings are then treated by 10 mixing and coating them with preheated bitumen in predetermined proportions of each; then during suction and agitation of the mass, subjecting the same to sustained heat sufficient to remove all moisture from 15 and to heat the particles; then mixing the coated stone, while hot, with the small particles and dust removed from the road's surface after coating such dust with atomized bitumen in said drum, and agitating 20 the same therein under sustained heat sufficient in duration and temperature to bring the temperature of the mass to approximately 250 deg. Fahr.; then depositing the same, in quantity merely sufficient to fill 25 the voids between the larger particles when compressed, onto said previously prepared surface while the latter is hot, then raking and compressing the same into shape, substantially as described.
- 30 2. The process of making a pavement consisting in heating a road's surface and removing the dust therefrom by suction thereof to a drum in which it is incorporated within new aggregate after being 35 coated with atomized bitumen therein and then mixed with stone of larger sizes coated in the absence of dust with hot bitumen under sustained heat sufficient to raise the temperature of the mass to approximately 40 250 degrees Fahr., then depositing the mass onto the heated surface, after spraying such surface with hot bitumen, and raking and compressing the same into shape.
3. The method of treating a worn surface of mineral matter, consisting in breaking it, then scarifying it, then creating a circular draft of hot air thereover by applying thereto flame under pressure, sucking such flame and hot air through flues 45 into a drum above the surface under treatment by means of fans operated by the mechanism of the self-propelled machine treating such surface, there being provided a plurality of such flames, flues and fans, 50 which latter also conduct such hot air from the drum back to the road's surface and within the influence of said suction during movement of the machine over the surface, thereby creating a sheet of flame and hot 55 air of which the plurality of flames form a part; simultaneously heating the surface while removing therefrom mineral matter of sizes smaller than those that pass a screen containing 80 mesh to the linear inch; 60 entrapping the latter in atomized bitumen

in the drum and mixing the same with precoated stone under sustained heat sufficient to raise the temperature of the mass to approximately 250 degrees Fahr., and to drive off all moisture therefrom; then depositing the same onto said dustless, heated stone on the road, pre-penetrated by heated bitumen, and pressing the same to substantial density, substantially as described. 70

4. The method of heating a bituminous 75 mixture for road paving purposes, consisting in first mixing cold aggregate with pre-heated bitumen; then mixing preheated impalpable dust with preheated bitumen, and mixing the ingredients together in a drum 80 heated externally by hot bitumen surrounding it, and the coated mixture directly under sustained heat from the supply thereof that heats the bitumen surrounding the drum; then agitating the mass under such sustained 85 heat until it reaches a uniform temperature of approximately 250 deg. Fahr.

5. The process of forming a paving structure in which the major portion of the aggregate is that of a worn structure of which 90 it forms a part, consisting in first scarifying the latter's worn surface to a substantial depth thereof, then directing, in a closure, hot air and flame under pressure thereagainst; then harrowing the surface, and 95 then blowing a plurality of flames from the rear of the machine forward of such surface in said closure during movement of the machine over such surface; then sucking the loosened and heated dust from the surface 100 and interstitial spaces of such structure to and within a preheated drum, and mixing the same with preheated bitumen-coated mineral particles; then forcing into said surface a predetermined quantity of hot bitumen; then 105 depositing the mixed material thereon, and compressing the same into shape, substantially as described.

6. The method of treating a wearing surface of a worn roadway by heating the same 110 with a blast of flames and hot air, simultaneously removing, by vacuum suction, the dust from its surface and interstices between its aggregate, and then forcing hot bitumen into such interstices by power distribution 115 of said bitumen, entrapping the dust in a drum therefor provided, and mixing the same with preheated bitumen, and then mixing the mass with bitumen-coated particles of relatively small size compared with those 120 of the old surface on which they are to be spread; then spreading the same onto said surface while the latter is hot and then compressing the same into shape.

7. A new paving structure comprising 125 relatively large sizes of stone coated in the absence of dust with bitumen and then bound with a mixture of mineral particles coated with bitumen of different consistency, in the absence of dust, mixed with bitumen-coated 130

dust acting as a filler colloidally interposed in all interstitial spaces between the coated particles, and compressed into shape.

8. The process of producing a filler for pavement aggregates consisting in mixing preheated impalpable dust in agitated air suspension with mineral matter and pre-heated bitumen in a drum while dehydrating the aggregate under the influence of suction and sustained heat during agitation of the mass, substantially as described.

9. The process of producing a bituminized stone and dust aggregate for paving purposes consisting in mixing moist stone particles of relatively small sizes in the absence of dust with a hard bituminous compound which has been reduced to a temporary liquid; then subjecting the mixture to sustained heat during agitation of the mass in an open ended vat, to convert the moisture in the stone into steam and to impregnate the stone with the bitumen during elimination of the steam from the vat by suction; simultaneously spraying impalpable dust in air and steam suspension in said vat with atomized bitumen of relatively low penetration and then agitating all of the ingredients together within said vat; then removing the same from the vat and spreading the same

over, and then compressing the same within, interstices between loosened stone of relatively large sizes preheated and bituminized in the absence of dust, while all of the ingredients are hot.

10. The process of making a pavement consisting in scarifying, heating, and removing impalpable dust from the surface and interstices of, stone constituting macadam paving structures; then coating the aggregate thereof *in situ* with a heated bituminous compound; then spreading thereover a matrix consisting of approximately thirty three per cent. by volume of the completed structure, composed of bituminized stone screenings containing in excess of fifteen per cent. of impalpable dust precoated with bitumen, and then pressing the matrix down and within the open interstices of the macadam structure and consolidating the same by rolling, while all of the ingredients are hot. 50

In testimony whereof I have affixed my signature in the presence of two witnesses this fourteenth day of January, 1918.

GEORGE A. HENDERSON.

Witnesses:

F. L. ALFORD,  
R. C. SWEET.